

## UNITED STATES PATENT OFFICE

2,030,767

## PROCESS FOR IMPROVING MAGNESIUM ALLOYS, ESPECIALLY IN SHAPED FORMS

Walther Schmidt, Paul Spitaler, and Werner Schultze, Bitterfeld, Germany, assignors, by mesne assignments, to Magnesium Development Corporation, a corporation of Delaware

No Drawing. Application August 11, 1932, Serial No. 628,294. In Germany April 25, 1929

## 2 Claims. (Cl. 148—21.3)

This invention relates to processes of improving magnesium base alloys and particularly to such processes when practiced in connection with magnesium base alloys containing substantial amounts of an alloying element which is capable of forming with the magnesium a solid solution. This application is a continuation in part of our application Serial No. 447,098, filed April 24, 1930.

Among the processes of treating magnesium base alloys to modify or develop properties in the metal, heat-treatment is the most important. The magnesium base alloy is usually subjected to a heat-treatment which comprises heating the metal to a relatively high temperature, such as a temperature somewhat below that temperature at which the most fusible constituent of the alloy melts, and thereafter quenching the thus heated article. After quenching, it is usual to submit the article to an aging treatment which comprises heating it for extended periods of time at temperatures below about 300° centigrade. By means of such a process there is first established in the magnesium base alloy a state of equilibrium at high temperature. By quenching the magnesium base alloy, this state of equilibrium is retained at normal temperatures. The subsequent aging of the alloy causes the establishment in the alloy of a state of equilibrium corresponding to a lower temperature; that is to say, the conditions produced at high temperature and retained by quenching are partially destroyed by the aging treatment. The result of the aging is a hardening effect in the alloy as well as improvements in other properties of the metal. When processes of heat-treatment such as the one above described are applied to magnesium base alloy castings, the quenching operation sets up stresses in the castings which, under some conditions and particularly in the case of complicated castings, may lead to the formation of cracks. Likewise, in most cases, these stresses tend to relieve themselves either at once or after the castings are machined or in use, with the result that distortion or warping of the casting takes place to such an extent that in some cases the castings will not serve the purpose for which they were intended.

The methods of this invention comprise improving magnesium base alloys containing between about 1 and about 15 per cent of alloying constituent which forms a solid solution with magnesium and which increases in solubility in the magnesium as the temperature of the alloy is increased, comprising heating the alloy to above about 325° centigrade but below the tem-

perature at which the most fusible constituent of said alloy fuses, and thereafter cooling said alloy through the temperature range of 300° centigrade to at least 100° centigrade at an average rate of not more than about 66° centigrade per hour.

In order to produce a state of equilibrium which is stable at high temperatures, the castings are first subjected to a heat-treatment above about 350° centigrade but below the temperature at which the most fusible constituent of said alloy fuses. In commercial practice it is preferable to heat-treat at a temperature which is but a few degrees below the temperature at which the most fusible constituent of the alloy fuses, but heat-treatment within the range defined will produce results. This heat-treatment having been completed in a manner well known to the art, the alloy is then cooled to room temperature or to normal temperatures at a rate which is considerably slower than that rate of cooling undergone when the alloy is allowed to cool in the open air. We have determined that it is particularly important to retard the cooling in the temperature range from about 300° to 100° centigrade, and we have further determined that in order to produce the most desirable results, the average rate of cooling between the temperatures of 300° and 100° centigrade should not be more than about 66° centigrade per hour.

The duration of the cooling in the temperature range below 100° centigrade is, according to our discoveries, of less vital importance, and retarded cooling need not be practiced throughout this range.

As a result of the practice of the methods of our invention, the castings produced are relieved of the stresses and strains which have hitherto been present in such castings when they were treated according to the prior methods above described. Moreover, this effect has been achieved without a material loss of the beneficial properties induced by heat-treatment in magnesium base alloys of this character.

The magnesium base alloys to which this invention refers are those alloys containing at least about 70 per cent of magnesium and about 1 to 15 per cent of alloying constituent which forms a solid solution with magnesium and which increases in solubility in magnesium as the temperature of the alloy is increased. Among such alloying elements are aluminum, tin, lead, manganese, zinc, etc. Of these alloys, magnesium base alloys containing aluminum are particularly useful commercially, and the methods of our in-

vention will find immediate commercial application in connection with magnesium alloys containing about 4 to 14 per cent of aluminum; the magnesium base alloys containing 6 to 12 per cent of aluminum being the magnesium-aluminum alloys in which the effect of our novel methods of treatment is most pronounced. Other commercial alloys containing tin or manganese or lead or zinc or combinations of these elements among themselves or with aluminum are likewise materially benefited when the heat-treatments above described are practiced in connection therewith. For instance, good results are obtained in the case of magnesium base alloys containing 6 to 10 per cent of tin or 0.5 to 6 per cent of zinc and, in fact, in connection with any of the magnesium base alloys in which the older methods of heat-treatment have caused improved properties. To the magnesium base alloys containing the solid solution-producing alloying elements of the class above described may be added one or more other alloying elements such as calcium, copper, barium, silicon, antimony, nickel, cadmium, etc., which impart to such alloys useful properties or modify some property of the alloy.

As an example of the practice of the methods of our invention in connection with a highly useful magnesium base alloy may be cited the following:

Castings of a magnesium alloy containing about 8.2 per cent of aluminum were heated at 410° centigrade for 72 hours and then cooled to 100° centigrade—in one case during 24 hours, and in another during 48 hours—in a furnace protected against radiation, or heated, the temperature drop being so arranged that the time allowed, in the latter case, for traversing the temperature zone between 300° and 100° centigrade, was about twice as long (namely, about 40 hours) as in the former case (about 18 hours). By means of this treat-

ment, the following values for the mechanical properties were obtained:

|                                  | Kz.<br>Kg./sq.<br>mm. | Elonga-<br>tion<br>Percent | Contraction<br>Percent | Elastic limit<br>Kg./sq.<br>mm. | Yield point<br>Kg./sq.<br>mm. | 5<br>10<br>10 |
|----------------------------------|-----------------------|----------------------------|------------------------|---------------------------------|-------------------------------|---------------|
| Original condition               | 16.6                  | 2.7                        | 1.8                    | 4.7                             | 10.3                          |               |
| Heated and cooled during 24 hrs. | 23.3                  | 5.6                        | 7.5                    | 6.0                             | 12.0                          |               |
| Heated and cooled during 48 hrs. | 23.6                  | 3.4                        | 5.0                    | 7.4                             | 13.9                          |               |

Although the advantages of our invention are primarily manifest in the case of castings, the invention is also applicable to magnesium base alloys of the class described which have been shaped when hot such as by rolling, extruding, drawing, forging, etc.

Having thus described our invention, what we claim is:

1. A process for improving the physico-mechanical properties of a magnesium alloy containing about 8.2 per cent of aluminum, which process comprises heating the alloy at 410° C. for 72 hours and then cooling the alloy down to 100° C. in a furnace within about 24 hours, the temperature drop being so arranged that the time allowed for traversing the temperature zone between 300° and 100° C. is at least about 18 hours.

2. A process for improving the physico-mechanical properties of a magnesium alloy containing about 8.2 per cent of aluminum, which process comprises heating the alloy at 410° C. for 72 hours and then cooling the alloy down to 100° C. in a furnace within about 48 hours, the temperature drop being so arranged that the time allowed for traversing the temperature zone between 300° and 100° C. is about 40 hours.

WALTHER SCHMIDT.

PAUL SPITALER.

WERNER SCHULTZE.